

Sept. 22, 1959

W. K. T. GLEIM

2,905,624

MANUFACTURE OF LUBRICATING OIL

Filed Nov. 7, 1955



INVENTOR:  
William K. T. Gleim

By: Chester J. Giuliani  
ATTORNEY:  
Glen R. Grunewald  
AGENT:

1

2,905,624

## MANUFACTURE OF LUBRICATING OIL

William K. T. Gleim, Island Lake, Ill., assignor, by mesne assignments, to Universal Oil Products Company, Des Plaines, Ill., a corporation of Delaware

Application November 7, 1955, Serial No. 545,262

10 Claims. (Cl. 208—89)

This invention relates to a process for the manufacture of lubricating oil and in particular to a novel process for treating a petroleum fraction to recover a lubricating oil therefrom which has properties superior to presently available lubricating oils.

As a general rule the components of a petroleum fraction which possess lubricating properties are the paraffinic and isoparaffinic hydrocarbons. Aromatic or alkyl-aromatic hydrocarbons destroy the lubricating quality of an oil fraction containing them and are therefore undesirable. The normal paraffinic constituents of a lubricating oil have a higher melting point than the isoparaffinic constituents and therefore yield oils which have poor temperature characteristics in spite of good lubricating characteristics. Condensed ring naphthenic compounds have poor lubricating properties and also have an adverse effect on the viscosity index of the oil. Naphthenic compounds which boil in the lubricating oil range and which are not condensed have no pronounced effects.

Previous treatments of petroleum fractions to produce lubricating oils have consisted largely of a separation of aromatic hydrocarbons from nonaromatic hydrocarbons which is followed by dewaxing, the latter process removing high molecular weight normal paraffinic constituents that are normally solid, followed by color improving processes such as clay treating or acid washing. The lubricating oil thus produced has reasonable lubricating properties being rich in isoparaffinic compounds, but the condensed ring naphthenic compounds give it poor viscosity characteristics and chemical instability.

Although an oil has good lubricating properties as manufactured, when it is used, for example, in a crankcase it is subjected to high temperature contact with metals such as iron, chromium, molybdenum, nickel, etc., which metals, although used structurally as components of iron and steel, still retain their well-known catalytic properties. In addition to being in contact with these catalytic materials, the crankcase is filled with oxygen, nitrogen, and other constituents to be hereinafter described. The original petroleum fraction usually contains small amounts of impurities such as hydrocarbon molecules with combined sulfur, nitrogen, oxygen, halogen, or other material. These materials may decompose under the conditions in the crankcase to form oxides or hydrides of the non-hydrocarbon portion of the molecule thereby introducing into the crankcase such materials as sulfur oxides, nitrogen oxides, water, hydrogen sulfide, etc. As a result, corrosive acid solutions are present during the operation of the vehicle with the well-known effect upon engine parts.

The presence of acidic materials and catalytic metals at high temperature in the crankcase of an automobile will cause the conversion of hydrocarbons. A most readily effected conversion at these conditions is the dehydrogenation of polynuclear naphthenic compounds to form their corresponding aromatic compounds and other reactions which may occur include cracking, condensation reactions and others. These reactions or any com-

2

bination of them will obviously change the composition of the oil.

The condensation reactions, besides changing the composition of the oil, cause the formation of heavy material which is generically known as sludge. This extremely viscous or solid material fouls the valves and piston rings of the engine.

It is an object of this invention to prepare a lubricating oil that not only has superior lubricating qualities but is prepared by a specific combination of steps to anticipate crankcase conditions and retain good lubricating qualities during use. This object is accomplished by treating an oil fraction with a combination of specific steps to regulate its composition to contain only constituents which have good lubricating qualities and leave out those which form undesirable material.

In line with accomplishing this object, it has been observed that condensed ring naphthenes have very poor viscosity characteristics and poor lubricating qualities. These compounds dehydrogenate easily to form condensed ring aromatic compounds which in turn condense further to form gum, tar, varnish, carbon or sludge as hereinbefore described.

It is, therefore, an embodiment of this invention to provide a process for the manufacture of lubricating oil which comprises contacting a hydrocarbon oil fraction boiling above 550° F. with a non-acidic supported hydrogenation catalyst in the presence of hydrogen at conditions to cause dehydrogenation of condensed ring naphthenic compounds, separating the resultant material into aromatic and nonaromatic fractions and recovering the desired lubricating oil from said nonaromatic fraction.

In a more specific embodiment this invention provides a process for the manufacture of lubricating oil which comprises contacting a hydrocarbon oil fraction boiling above 550° F. with a desulfurization catalyst in the presence of hydrogen at superatmospheric pressures and at desulfurizing conditions, separating the desulfurized material into a normally liquid and a normally gaseous fraction, passing the liquid fraction into contact with a hydrogenation catalyst supported on a non-acidic base in the presence of hydrogen at conditions to cause dehydrogenation of condensed ring naphthenic compounds, separating the resultant material into aromatic and nonaromatic fractions and recovering the desired lubricating oil from said nonaromatic fraction.

The process of this invention may be better described with reference to the accompanying drawing which shows a flow diagram of the process in schematic form. This description is not intended as limiting upon the invention but only as being illustrative thereof and it is intended that all equivalent substitutions of one means for another are included within its broad scope.

The charge stock passes through line 1 to impurity removal zone 2. This charge stock is a hydrocarbon fraction preferably boiling between 550 and 950° F. and at least in excess of 500° F. Its source will usually be petroleum which will usually be a selected fraction distilled from a crude, but may be previously treated material such as cycle stock, however, the fraction may be obtained from the distillates resulting from coke production or from shale, oil sands or any other source of hydrocarbon material. It is preferred when producing lubricating oil that the charge stock be a paraffinic petroleum fraction or at least a fraction that has been deasphalted prior to treatment by such means as propane deasphalting. It is usually desirable to dewax the charge to the process prior to this treatment for the purpose of removing material from the process which will not be benefited by the process and for the purpose of recovering the wax, which is a valuable product in its own right.

The charge stock passing into the impurity removal zone 2 is first heated to a temperature of between 400° F. and 650° F. and commingled with a hydrogen-containing gas at a pressure of from about 200 p.s.i. to about 1000 p.s.i. or more. The desulfurizing zone will contain a catalytic material which is adapted to desulfurization. Such materials generally are compounds having hydrogenation activity but which are resistant to sulfur poisoning. Typical of such materials are the metals of group VI and group VIII of the periodic table which are catalytic in the form of the elemental metal and in the form of its oxide or sulfide. As is well known in the chemical art, catalysts employing these rather valuable metals can be made with great economy of material without sacrificing activity by disposing the metals on a suitable inorganic oxide support having high surface area and adsorptivity. Therefore, the preferred catalyst for use in impurity removal zone 2 is a metal such as tungsten, cobalt, molybdenum, chromium or mixtures thereof, preferably mixtures of cobalt and molybdenum disposed on a porous inorganic oxide support such as silica, alumina, zirconia, magnesia or combinations thereof, but preferably alumina or alumina stabilized with a small amount of silica.

The petroleum fraction passing through the impurity removal zone at the stated conditions is substantially unchanged by the contact with a catalytic material in all respects except that its composition with regard to sulfur, nitrogen and oxygen is drastically reduced. The impurity removal zone causes the molecules bearing sulfur, nitrogen or oxygen to decompose into hydrogen sulfide, ammonia and water and the corresponding saturated hydrocarbons. The impurity removal zone will also contain means for separation of the normally gaseous from normally liquid material resulting from this zone and will pass the normally liquid material via line 3 to hydrogenation and dehydrogenation zone 4. The normally gaseous material from impurity removal zone 2 may be vented, recirculated or partially vented and partially recirculated as the economy of the process dictates.

Hydrogenation and dehydrogenation zone 4 contains a catalyst having high hydrogenation activity supported on a non-acidic base. This composite catalyst results in a catalyst which will have activity only towards dehydrogenating and hydrogenating hydrocarbons but will not promote cracking, dehydrocyclization or dealkylation reactions. This catalyst is preferably a supported platinum or palladium catalyst with a support comprising a non-acidic base. A non-acidic base may consist of such inorganic oxides as alumina, silica, zirconia, magnesia, naturally occurring clays, kieselguhr or mixtures such as silica-alumina, silica-magnesia, etc., however, these materials if not catalytically inert by nature should first be treated with steam, alkali carbonate, hot water or ammonia or other reagents to deactivate them. To avoid destroying the high surface area of the base, it is preferable to composite it with alkaline or alkaline acting material such as alkali metal oxides, alkaline earth metal oxides, amines, ammonia or the like to impart thereto an alkaline quality thereby insuring a lack of acidity. Another suitable base material may be carbonaceous in nature such as coke, coal, activated charcoal, etc., which material generally has high adsorptive qualities but which is inert regarding cracking or catalytic qualities.

The metal constituent having high hydrogenating activity which may be platinum, palladium, nickel, cobalt, molybdenum, tungsten, etc., but preferably platinum or palladium, may be composited with the non-acid base by any of the well-known means such as by impregnating the base with a solution of a soluble salt of the catalytic metal, drying and calcining the thus impregnated base to result in the deposition of the oxide of the catalytic metal thereon.

Hydrogenating and dehydrogenating zone 4 is maintained at carefully controlled conditions to cause the de-

hydrogenation of condensed ring naphthenes and the hydrogenation of unsaturated aliphatic compounds. By contacting the hydrocarbon with the catalyst in the presence of hydrogen at a temperature of from about 500 to about 900° F., the desired reactions may be effected when using an active catalyst such as platinum or palladium. When a desulfurization zone, as in this embodiment, precedes the hydrogenation and dehydrogenation zone, a highly active but impurity-sensitive catalyst such as platinum or palladium may be employed over long periods of time without adverse effects.

The material passing from hydrogenation and dehydrogenation zone 4 will consist of paraffinic and isoparaffinic hydrocarbons in substantially the same condition as when they entered the process. If the charge to the process contains unsaturated aliphatic material, this will be saturated and will become part of the paraffinic and isoparaffinic hydrocarbons. Non-condensed naphthenic compounds or paraffinic compounds with naphthenic side chains are not as readily dehydrogenated as condensed ring naphthenes which will be dehydrogenated to form aromatic or alkyl aromatic compounds. The effluent may also contain hydrogen gas and some lower boiling hydrocarbons such as those boiling in the kerosene, gasoline or lower boiling range which result from a small amount of cracking or dealkylation. The total effluent is passed to a receiver and separated into a normally gaseous fraction and a normally liquid fraction. The normally gaseous fraction may be recycled at least in part to the hydrogenation and dehydrogenation zone and the normally liquid portion passed through line 5 to aromatic separation zone 6.

In aromatic separation zone 6, a separation by hydrocarbon type is effected to remove aromatic hydrocarbons and unsaturated hydrocarbons from the naphthenic and paraffinic hydrocarbons. This separation is preferably effected by absorption on a solid such as silica gel, activated charcoal, etc., or liquid-liquid extraction process wherein the hydrocarbon phase is contacted with a substantially immiscible liquid phase which is a selective solvent for aromatic hydrocarbons. Suitable solvents may include  $\text{SO}_2$ , HF,  $\text{AlCl}_3$ ,  $\text{H}_2\text{SO}_4$  and other materials that tend to condense unsaturates but preferably the solvent will comprise a material chemically inert with respect to the hydrocarbon. The solvent may comprise organic liquids such as glycols, methanol, aldehydes, nitriles, dinitriles, amines, etc.

Substantially complete removal of high boiling aromatics may be effected by selective adsorption wherein an adsorptive solid which selectively adsorbs aromatic and unsaturated hydrocarbons is commingled with the oil. These processes may be effected continuously or with a fixed bed of material such as silica gel, activated charcoal, Attapulgus or other clays or similar materials. When a selective adsorption process is employed for aromatic removal, it may not be necessary to provide for separate sulfur removal since the selective adsorbent will remove most of the sulfur-bearing molecules in the liquid. Other means of removing the aromatic material is by converting it chemically to a more readily removable form. Therefore, treating the entire fraction with certain nitrogen-containing organic compounds such as trinitrotoluene or picric acid will cause a solid phase containing aromatic material to precipitate and acid-washing with sulfuric acid will remove the aromatic material. The preferred modes of aromatic separation are by adsorption on a solid and by solvent extracting with a selective solvent. These modes are preferred since the aromatic materials separated are not destroyed and may find other uses, and since substantially complete aromatic removal may be economically effected.

The nonaromatic portion from aromatic separation zone 6 passes through line 7 to finishing zone 8. In finishing zone 8 whatever processes are required to make a complete product from the material in line 7 are ef-

fected. The processes may include, for example, fractionating the resultant lubricating oil into its various grades such as SAE 10, SAE 20, etc., and making suitable blends for specific purposes. Since the process of this invention produces a clean, colorless oil it is not necessary to employ a clay treating or acid treating step in the finishing. The finishing zone may also include a dewaxing stage to remove wax if it has not been previously removed or to remove wax which is formed in the process, for example, by hydrogenation of an unsaturated aliphatic molecule which was olefinic as part of the charge.

The lubricating oil resulting from this process will have excellent lubricating properties and, as will be hereinafter illustrated, the process of the present invention produces a product having superior temperature characteristics as will be indicated by the improved viscosity index of the product over the charge to this process. The viscosity index is an arbitrary measure indicating the rate of change of viscosity with temperature, with high viscosity index preferred to low viscosity index.

The following examples are presented to illustrate specific modes of operating the process of the present invention and are not intended as being unduly limiting upon the broad scope thereof.

#### Example I

A Mid-Continent crude oil was distilled and the fraction boiling between 550° F. and 950° F. was separated and dewaxed. This fraction was then blended with hydrogen in a proportion of 1500 standard cubic feet of hydrogen per barrel of liquid and the resultant mixture was heated to a temperature of 570° F. and passed into the top of a catalyst tube at a pressure of 350 p.s.i. The catalyst tube contained a bed of  $\frac{1}{8}$ " x  $\frac{1}{8}$ " cylindrical pellets of alumina which were impregnated with cobalt and molybdenum in a proportion of 4% by weight of cobalt and 8% by weight of molybdenum. The proportion of cobalt and molybdenum are based on the weight of actual metal present as compared with the weight of alumina in the catalyst and this stoichiometric measurement is intended to be for convenience of comparison rather than to indicate that the metals are in any particular form in the catalyst. The cobalt and molybdenum, which may be in the form of the pure metal, the oxide, the sulfide or mixtures of these, is disposed on the alumina pellets by soaking the pellets in solutions of the soluble salts of the metals and thereafter draining and drying the pellets thus impregnated. This impregnation may be successive, impregnating first with one and then with the other of the salts, or it may be accomplished simultaneously by impregnating with a single solution containing the salts of both metals.

The material passing from the desulfurization zone was separated into liquid and gas phases and the liquid which was stripped substantially free of hydrogen sulfide, ammonia and other normally gaseous material and passed over silica gel to remove aromatic compounds was introduced into a vessel containing a catalyst consisting of alumina pellets upon which 0.3 weight percent platinum was disposed by impregnating from a solution of chloroplatinic acid. The mixture of catalyst and oil was heated to a temperature of 650° F. and hydrogen at substantially atmospheric pressures was bubbled through this mixture from the bottom of the vessel.

The effluent from this reaction zone contains 10% aromatics and the rest of the material consists of paraffinic, isoparaffinic and alkylmononuclear naphthenic compounds.

The effluent from the hydrogenation and dehydrogenation zone was then passed into a tube containing silica gel and the effluent from the silica gel treatment was found to be substantially free of aromatic compounds. This product is water white and requires no further treatment, except fractionation into particular boiling ranges when desired.

The initial charge to the process contained 0.18 weight percent combined sulfur, 0.009 weight percent combined nitrogen and it had a viscosity index of 88.7. The product from this process contains 0.04 weight percent sulfur, it is virtually free of combined nitrogen and the viscosity index is 111.9. The product contains substantially no polynuclear material and is substantially inert to hydrogenation, dehydrogenation, dealkylation, cracking reactions and dehydrocyclization reactions at the conditions in a crankcase if combined with the proper additives.

#### Example II

In Example II the process of Example I was repeated in every detail except that the hydrogenation and dehydrogenation zone employed a catalyst comprising 2.0 weight percent palladium disposed on alumina instead of the platinum catalyst of the previous example. The process resulted in the production of 20% aromatics which upon removal with a silica gel column resulted in a product having a viscosity index of 113.11 instead of the viscosity index of 88.7 of the initial dewaxed charge.

#### Example III

The process of Examples I and II was repeated employing as a hydrogenation and dehydrogenation catalyst a composite of 0.3% platinum oxide on alumina. The hydrogenation and dehydrogenation process resulted in an aromatic production of 18.5 weight percent aromatics which upon removal resulted in a lubricating oil product having a viscosity index of 112.79.

#### Example IV

The process of the above examples was again effected only employing this time a catalyst in the hydrogenation and dehydrogenation zone containing 5 weight percent palladium impregnated onto activated charcoal. The product was treated by countercurrently contacting it with silica gel which resulted in the removal of the aromatic portion of the product and produced a raffinate substantially free of aromatics having a viscosity index of 110.8.

The products from all of the above experiments were commingled with various amounts of various viscosity index-improving additives to determine whether or not the response to such additive improvement was changed by this treatment. It was found in all cases that the improvement effected by the additive was unchanged, that is, the addition of 2% of a viscosity index-improving additive resulted in the same increment of improvement to the product of this process as to the charge. Therefore, the gain in viscosity index that is realized is a real gain which is not diminished by poor response to additives.

From the foregoing, it may be seen that the process of the present invention provides a means for preparing a clean, high grade lubricating oil which upon addition of conventional additives has excellent lubricating qualities and is composed to retain these qualities even though subjected to severe crankcase conditions in the presence of reaction promoting material. Furthermore, the product of this process has improved temperature characteristics over the charge stock.

When lubricating oil is referred to in the specification and appended claims, it is not intended to imply that the product from this process is a complete oil. It is, however, intended that well known detergents, oxidation inhibitors and other additives may be added to perform their usual functions.

I claim as my invention:

1. A process for the manufacture of lubricating oil which comprises contacting a hydrocarbon oil fraction boiling above 550° F. and containing condensed ring naphthenes with a hydrogenation catalyst supported on a non-acidic base in the presence of hydrogen at conditions to cause dehydrogenation of condensed ring naphthenic compounds to aromatics, separating the resultant ma-

terial into aromatic and nonaromatic fractions and recovering the desired lubricating oil from said nonaromatic fraction.

2. A process for the manufacture of lubricating oil which comprises contacting a hydrocarbon oil fraction boiling above about 550° F. and containing condensed ring naphthenes with a desulfurization catalyst in the presence of hydrogen at superatmospheric pressure and at desulfurizing conditions, separating the desulfurized material into a normally liquid and a normally gaseous fraction, passing the normally liquid fraction into contact with a hydrogenation catalyst supported on a non-acidic base in the presence of hydrogen at conditions to cause dehydrogenation of condensed ring naphthenic compounds to aromatics, separating the resultant material into aromatic and nonaromatic fractions and recovering the desired lubricating oil from said nonaromatic fractions.

3. The process of claim 1 further characterized in that said hydrogenation catalyst comprises platinum and alumina.

4. The process of claim 1 further characterized in that said hydrogenation catalyst comprises platinum deposited on a base of alumina and magnesium oxide.

5. The process of claim 1 further characterized in that said hydrogenation catalyst comprises platinum deposited upon a carbonaceous base.

6. The process of claim 1 further characterized in that said hydrogenation catalyst comprises palladium impregnated alumina.

7. The process of claim 1 further characterized in that said dehydrogenation is effected at a temperature of from about 500° F. to about 900° F.

8. The process of claim 2 further characterized in that said desulfurization is effected at a temperature of from about 450° F. to about 600° F.

9. The process of claim 2 further characterized in that said desulfurization catalyst comprises cobalt, molybdenum and alumina.

10. A process for manufacturing lubricating oil which comprises contacting a hydrocarbon oil fraction boiling above about 600° F. and containing condensed ring naphthenes with a desulfurization catalyst comprising cobalt, molybdenum and alumina in the presence of hydrogen at superatmospheric pressure and at a temperature of from about 450° F. to about 600° F., separating the desulfurized material into a normally liquid and a normally gaseous fraction, passing the normally liquid fraction into contact with a hydrogenation catalyst comprising platinum supported on alumina and magnesium oxide at a temperature of from about 500° F. to about 900° F. in the presence of hydrogen to convert the condensed ring naphthenes to aromatics, separating the resultant material into aromatic and nonaromatic fractions and recovering the desired lubricating oil from said nonaromatic fraction.

#### References Cited in the file of this patent

#### UNITED STATES PATENTS

|    |           |               |               |
|----|-----------|---------------|---------------|
| 20 | 1,908,286 | Dorrer        | May 9, 1933   |
|    | 1,955,861 | Russel et al. | Apr. 24, 1934 |
|    | 2,423,176 | Cole          | July 1, 1947  |
| 25 | 2,602,772 | Haensel       | July 8, 1952  |
|    | 2,697,682 | Porter        | Dec. 21, 1954 |
|    | 2,755,225 | Porter et al. | July 17, 1956 |
|    | 2,779,713 | Cole et al.   | Jan. 29, 1957 |

#### FOREIGN PATENTS

|    |           |        |               |
|----|-----------|--------|---------------|
| 30 | 1,064,400 | France | Dec. 23, 1953 |
|----|-----------|--------|---------------|

#### OTHER REFERENCES

35 Rossini et al.: Progress in Petroleum Technology (ACS #5), 1951, Amer. Chem. Soc., Wash., D.C., pp. 334-352 (p. 350 only relied on).